

# UNITED STATES PATENT OFFICE.

CHARLES ALMY, JR., OF WILMINGTON, DELAWARE, ASSIGNOR TO AMERICAN VULCANIZED FIBRE COMPANY, OF WILMINGTON, DELAWARE, A CORPORATION OF DELAWARE.

## PROCESS OF PURING HARD OR VULCANIZED FIBER.

1,191,142.

Specification of Letters Patent.

Patented July 18, 1916.

No Drawing.

Application filed March 19, 1913. Serial No. 755,413.

*To all whom it may concern:*

Be it known that I, CHARLES ALMY, Jr., a citizen of the United States, residing at Wilmington, in the county of New Castle 5 and State of Delaware, have invented certain new and useful Improvements in Processes of Puring Hard or Vulcanized Fiber, of which the following is a specification.

This invention relates to the manufacture 10 of so-called hard or vulcanized fiber and similar products and particularly to the so-called puring processes, the object of the invention being to provide a highly expeditious and economical process of this character.

It is well known that following the preparation of laminated sheets or tubes of vulcanized fiber by the action of strong zinc chlorid solutions upon suitable forms of cellulose paper, it is necessary to subject the product to a prolonged puring or washing process for the removal of the excess of zinc chlorid. As heretofore usually practised, the puring process involves subjecting the vulcanized fiber to a plurality of baths of zinc chlorid solution of progressively diminishing concentration, followed by a plurality 20 of washings with pure water. The time required for puring depends largely upon the thickness of the laminated sheet, and in many cases approximates ten days for each one-sixteenth inch in thickness; so that sheets having a thickness of three-eighths inch may require about two months for puring. 30 According to the present process, the time required for puring is greatly shortened, especially in case of the thicker sheets.

Careful analytical investigations of the removal of zinc chlorid by the puring process, as heretofore practised, have shown that the elimination of zinc chlorid is at first quite rapid, becoming however slower and slower as the treatment proceeds; and that the removal of the final portions of the salt to 40 attain the desired minimum percentage is extremely slow. For example, I have found that in the case of a sheet three-eighths inch in thickness, the percentage of zinc chlorid, based upon the weight of dry fiber, was reduced, in thirty days, from 130 per cent. to

about 1.0 per cent.; and that it required some thirty days additional treatment to reach the desired ultimate percentage of .02 to .08 per cent.

According to the present process, the hard or vulcanized fiber or similar material, prepared in any usual or desired manner, and in the form of sheets, tubes or other articles, is subjected to the usual treatment with zinc chlorid solutions of progressively diminishing concentration until the greater part of the zinc chlorid has been eliminated, and preferably until the residual chlorin is present in the proportion of less than one per cent. of the dry vulcanized fiber. At this stage, the product is submitted to an evaporative or drying process, as a result of which the residual zinc chlorid is largely carried, by capillary action, to the surface or superficial portions of the sheet. The sheet is then washed in pure water one or more times. By this treatment, a large proportion of the residual zinc chlorid is very quickly removed, and a product is obtained having the desired low percentage of the salt. The saving of time thereby effected is in all cases material, and in the case of the heavier sheets may amount to many days.

It is to be understood that while I have referred specifically to zinc chlorid solutions, the process is directly applicable to other solutions capable of giving similar results, as for example solutions of other salts of zinc, or solutions containing ingredients other than zinc salts.

A specific illustrative example of the new process is as follows: A vulcanized fiber sheet seven-eighths inch in thickness in the wet condition, was washed as usual in zinc chlorid solutions of diminishing concentration until the average chlorin-content was reduced to about 0.5 per cent. of the dry mass. The sheet was then heated at a temperature of 65 to 80° C., until its moisture-content was reduced to approximately ten per cent. An analysis of the resulting partially-dried product showed at or near the surface 2.27 per cent. of chlorin, and in the interior or central portions 0.201 per cent. of chlorin. The sheet was then washed with

85

90

95

100

pure water at a temperature of 60 to 70° C., when it was found that the zinc chlorid was very rapidly removed, and that two washings sufficed to reduce the percentage of zinc chlorid to the desired commercial minimum.

The process as above described may of course be modified as desired, according to the thickness of the sheets or other articles and the proportion of salt which is regarded as permissible in the final product. A complete drying of the sheet, in the sense of expelling all moisture therefrom, preliminary to the final washing, is unnecessary and usually undesirable. An evaporation of as little as ten per cent. of the contained moisture showed, in certain cases, a marked effect, but in most cases it is preferred to reduce the moisture-content to 10 to 25 per cent. by weight of the fiber, as a preliminary to re-soaking.

The precise stage in the elimination of the zinc chlorid at which the sheet is subjected to the above-described evaporative treatment is not material to the invention, but it is preferred to introduce the evaporative treatment at such a point in the process that the concentration of the zinc chlorid in the interior or central portion of the sheet will, after the evaporation, approximate the desired final concentration. If this is done, the final washing is required to remove the zinc chlorid from the surface and superficial portions of the sheet only, and is therefore very quickly accomplished. Furthermore, the central portions of the sheet are not necessarily thoroughly soaked by the final washing, with the result that the final drying is expedited.

The new process presents many material advantages, among which may be mentioned the following:

(1) A material saving of time in the final washing, and also in the final drying, with the result of expediting the preparation of all sheets, and particularly the thicker grades.

(2) In the finished sheets, as heretofore prepared, the percentage of zinc chlorid is invariably higher at the surface of the sheet than in its interior portions; whereas in sheets prepared according to the present process the surface-content of zinc chlorid is usually lower than the interior-content, so that the proportion of zinc chlorid in the finished sheet usually diminishes from the center toward the surfaces. This is a distinguishing characteristic of sheets prepared according to the present process, and is distinctly advantageous as reducing the surface conductivity of the sheet, as well as its tendency to absorb moisture from the air, as compared with a similar sheet prepared by the prior processes and having the same average salt-content.

(3) An illustrative example of the composi-

tion of a sheet prepared according to the present invention is as follows:

*Finished sheet three-fourths inch thick.*

|                             |        |    |
|-----------------------------|--------|----|
| Average chlorin-content     | 0.116% | 70 |
| Superficial chlorin-content | 0.052% |    |
| Central chlorin-content     | 0.138% |    |

*Finished sheet seven-sixteenths inch thick.*

|                             |        |    |
|-----------------------------|--------|----|
| Average chlorin-content     | 0.115% | 75 |
| Superficial chlorin-content | 0.069% |    |
| Central chlorin-content     | 0.127% |    |

It is of course to be understood that this example is illustrative only, and that the percentages of salt may be made either greater or less than those above mentioned, according to the details of the treatment to which the article is subjected.

(3) A material saving of zinc chlorid or equivalent chemical is effected, owing to the fact that the proportion of water required for the final washing is so limited as to render it possible, in most cases at least, to return all of the resulting highly-dilute salt solution to the process.

I claim:

1. The process of puring hard or vulcanized fiber and similar products, which consists in washing the same with suitable puring solutions of progressively diminishing concentration, subjecting the fiber to an evaporative process, and thereafter washing and drying the same.

2. The process of puring hard or vulcanized fiber and similar products, which consists in washing the same with suitable puring solutions of progressively diminishing concentration, then subjecting the fiber to an evaporative process to induce a movement of the residual salt to or toward the surfaces thereof and to reduce the concentration of the salt in the central portion to about the desired minimum, and thereafter washing and drying the fiber.

3. In a process of puring hard or vulcanized fiber and similar products, the step which consists in subjecting the fiber to an evaporative process to induce a movement of the residual salt to or toward the surfaces thereof, before the final washing.

4. In a process of puring hard or vulcanized fiber and similar products, the step which consists in subjecting the fiber to an evaporative process to induce a movement of the residual salt to or toward the surfaces thereof and to reduce the concentration of the salt in the central portion to about the desired minimum, before the final washing.

5. In a process of puring hard or vulcanized fiber and similar products by repeated washings, the step which consists in subjecting the fiber to an evaporative treatment before the final washing.

6. A sheet or other article of hard or vulcanized fiber or like material characterized by the presence therein of the vulcanizing agent in proportion diminishing toward the surfaces of the sheet.

7. A sheet or other article of hard or vulcanized fiber or like material characterized by the presence therein of chlorin in

proportion diminishing toward the surfaces of the sheet. 10

In testimony whereof I affix my signature in presence of two witnesses.

CHARLES ALMY, JR.

Witnesses:

T. W. CAMPBELL,  
G. K. PARSONS.

Copies of this patent may be obtained for five cents each, by addressing the "Commissioner of Patents, Washington, D. C."